

Nov. 6, 1928.

1,690,960

S. YAMANAKA

POLISHING PAD

Filed July 7, 1927



INVENTOR:

SABURO YAMANAKA.

BY ATTY:

*Edward M. Kojima*

## UNITED STATES PATENT OFFICE.

SABURO YAMANAKA, LOS ANGELES, CALIFORNIA.

## POLISHING PAD.

Application filed July 7, 1927. Serial No 204,125.

This invention relates to an improved pad to be used for polishing and cleaning varnished surfaces and metal surfaces and for producing a glossy finish thereon, and further relates to the method of making the pad.

It is well known that in compounds and liquid preparations heretofore used in cleaning and polishing metal surfaces, the fact that they contain benzine or gasoline, renders them dangerous and objectionable in use. Some of them, while serving to clean the metal surfaces, leave the same liable to corrosion, and do not produce a polish thereon.

The device hereinafter described is convenient, and particularly rapid in its action, and is particularly free from corrosive effect.

The drawing illustrates a form of this invention which I have found to be desirable in use.

20 In the drawing, the figure is a perspective view of a polishing pad constructed in accordance with my invention.

The device consists of a substantially rectangular pad 2, having holes 3 extending laterally therethrough.

In the fabrication of this polishing pad, I first take a quantity of horn material, preferably deer horns, and bake them with a heat, and then powder them. To this horn material, I add powdered squid shell (designated by some as cuttle-bone) and to these ingredients I add powdered pumice stone; the proportions being: powdered horn, one part; powdered squid shell, two parts; and powdered pumice stone, seven parts. After mixing these ingredients, I add a quantity of gelatin, and again mix the same thoroughly into a paste. I then take a quantity of animal hair and cut the same into suitable lengths, and mix it with the gelatin paste. I then compress the same, and, after suitable drying, I cut the hair felt compound into suitable pads.

In use, the pad is dipped into water, and, after the surplus water is squeezed out, the pad is ready for use in polishing a metal surface, and also enameled wood and varnished surfaces.

The compound or mixture of the present invention possesses the qualities of effecting a uniform and perfect cleaning and brighten-

ing of metal surfaces when applied thereto and subjected to the necessary rubbing; producing a lustrous and glossy finish.

When used as specified, the water serves as 55 a vehicle for the other ingredients, and the gelatine and powdered pumice stone remove dirt without scratching or marring, although the pumice has abrasive properties. The powdered horn and powdered squid shell 60 produce a glossy and brilliant polish. The hair ingredient serves to retain the other ingredients in a relative mass or form, and the homogeneous pad thus formed efficiently cleans and polishes, and gives a more lustrous 65 finish, than can be obtained with ordinary cleaners, and the rubbing afterward with cloth or chamois skin.

The polishing pad thus fabricated, contains no acids, benzine, naphtha, or alkaline ingredients, and will not injure the hands of the user. In addition, the gelatine and other smoothing ingredients such as the powdered squid shell, deposit on the polished surface, an exceedingly thin film or coat which preserves the metal from corrosion. No limitation is made to the form of the pad shown in the drawing, as the same may be made any size or form desired without departing from the spirit of the invention. 70 75 80

What is claimed is:

1. A polishing pad, consisting of a body of hair felt having holes extending laterally therethrough, and polishing ingredients homogeneously compounded with the hair 85 felt.

2. A polishing pad, including a body of hair felt, and a compound incorporated therein, consisting of powdered horn; one part, powdered squid shell, two parts, powdered 90 pumice stone, seven parts, and gelatin.

3. The herein described composition of matter fabricated into a polishing pad, consisting of animal hair cut into short lengths, gelatin, powdered horn, powdered squid shell, 95 and powdered pumice stone, combined, substantially in the manner and in the proportions stated.

In testimony whereof, I hereunto affix my signature.

SABURO YAMANAKA.